

## UNITED STATES PATENT OFFICE

ERICH BÖHM, OF VIENNA, AUSTRIA

## PROCESS FOR TREATING ANIMAL HAIR AND WOOL WITH CHLORINE

No Drawing. Application filed November 22, 1927, Serial No. 235,125, and in Austria December 1, 1926.

My invention relates to an improved method of treating animal hair and wool with chlorine for preparing it for fulling and felting or, as it is called in manufacturing hats, 5 for carressing it.

It has already been proposed to treat animal hair and wool with hypochlorites, with chlorine water and even with gaseous chlorine for improving the lustre of the same. But 10 the methods heretofore used in such treatments resulted invariably in a highly objectionable action on the hair and wool viz: a reduction of the mechanical strength, and even a rapid destruction thereof and more 15 particularly a complete loss of the capacity of hair and wool to be fulled or felted.

The main object of my invention is to avoid the deleterious effects above referred to of the chlorine treatment of hair and wool and 20 to provide a method for such treatment which imparts to animal hair and wool the capacity of being readily fulled and felted or which improves this capacity without producing any deleterious effect on the hair or wool.

25 In carefully studying the action of chlorine on animal hair and wool I have discovered that any deleterious action of chlorine on animal hair and wool can be avoided by providing for a comparatively slow development of chlorine on the hair and wool itself, and avoiding the presence or formation of hypochlorites and hypochlorous acid, while the formation of chlorine dioxide ( $\text{ClO}_2$ ) appears to have even a beneficial effect. 30 By satisfying these conditions I make animal hair and wool particularly fit for fulling or felting. Thus for instance hair from hares and rabbits which cannot be fulled or felted without special preparation usually by nitric acid and mercury nitrate, such preparation being called carressing, is made fit for fulling and felting or carressed by my improved process in a very efficient manner.

40 Other kinds of animal hair or fibre such as certain coarse kinds of wool, for instance cross-bred wool, which could not be made fit for felting or fulling by any known methods, may be readily worked into felt hat bodies after having undergone my improved chlorinating process.

With the object above referred to in view, my improved process comprises the step of applying to the animal hair or wool either on the skin or after cutting, an aqueous solution of a chloride and an aqueous solution of an oxygen carrier capable of liberating chlorine from the said chloride. 55

The concentrations of the said aqueous solutions are so weak, that when cold no reaction is set up between them by which chlorine is liberated, but such reaction is set up on heating the mixture of the said aqueous solutions to from 50 to 100° centigrade. Or this reaction may be set up on increasing the concentration of the mixture of the said aqueous 60 solution by evaporation. 65

I may apply the said aqueous solutions to the hair or wool to be treated in any suitable or preferred manner, either simultaneously or successively by spraying or by brushing or by simply immersing the hair or wool to be treated into the said solutions successively or preferably into the mixture of such solutions and subsequently removing the excess liquid by pressing or by centrifugal action. Or I 70 may simply immerse the hair and wool into the mixture of the aqueous solutions and then heat the whole to a temperature of 50 to 100° centigrade. 75

The chlorides used in my improved process are inorganic or organic chlorides including hydrogen chloride or hydrochloric acid, or mixtures of substances capable of producing such chlorides. The oxygen carriers may be peroxide of hydrogen persulphuric acid, 80 persulphates, chloric acid, chlorates or other substances rich in oxygen and capable of liberating chlorine from chlorides. 85

In some cases I may use besides the aqueous solutions of chlorides and oxygen carriers 90 also acidulating agents, that is to say aqueous solutions of acids other than those serving as oxygen carriers or salts showing a reaction in aqueous solutions for enhancing or facilitating the liberation of chlorine. Such acidulating agents are oxalic or tartaric acid and even nitric acid or salts of iron, copper, nickel, cobalt chromium, manganese, molybdenum or tungsten. 95

In either case of heating or of drying the 100

aqueous solutions in contact with the hair or wool, the chlorine is immediately taken up by the hair or wool as it is liberated and as the chlorine accompanied or not by chlorine dioxide is liberated comparatively slowly, any deleterious action on the hair or wool is avoided.

If the said aqueous solutions are applied to the hair or wool on the skin by spraying 10 or by brushing or by immersion and subsequent removal of the liquid in excess, the quantity of chlorine liberated on and taken up by the hair or wool may be nicely predetermined.

15 If cut hair or wool has to be treated by my improved process I prefer to simply immerse it in the mixture of the said aqueous solutions and then to heat the whole to a temperature of 50 to 100° centigrade.

20 If my improved process has to be carried out in the last named way by simple immersion and subsequent heating, the concentration of the aqueous solutions is preferably much lower, about only one fifth to one 25 twentieth of that used in the former case.

The aqueous solutions above referred to are of a comparatively low concentration. The percentage of chlorine capable of being liberated in such mixtures of aqueous solutions may vary from one tenth to three percent, the quantity of the oxygen carrier in the mixture of solutions is such as to enable the said quantities of chlorine to be liberated from the chlorides. In the said quantities 35 of chlorine those contained in the readily decomposing chlorine dioxide if such be formed are included.

I wish it to be understood that hypochlorous acid or hypochlorites are not included in 40 the chlorides used according to my invention.

#### Examples

(1) Cut hair or wool is immersed for about 1/2 hour into a bath consisting of an aqueous solution containing 0.05 to 0.2% of hydrochloric acid as a chloride and 0.25 to 45 1% of peroxide of hydrogen or an oxygen carrier to which 0.01%–0.1% of a salt as above described for instance copper sulphate 50 or manganese chloride may be added. After removing the excess of liquid the hair or wool is dried at a temperature of 70 to 100° centigrade. It will be found that the hair or wool thus treated is thoroughly carotted.

55 (2) To hair or wool on the skins is applied by spraying or brushing an aqueous solution containing 1% of potassium chlorate and 3% of hydrochloric acid and then the 60 skins so treated are dried at a temperature of 70 to 100° centigrade. The hair or wool thus treated is not only thoroughly prepared for fulling and felting or carotted, but also shows a very beautiful durable lustre. The 65 effect of this bath may be notably enhanced

by adding thereto 0.5 to 1% oxalic acid or tartaric acid as an acidulating agent.

I prefer to use uncoloured chlorides and oxygen carriers. Thereby I avoid any discolouring of the hair or wool which is more particularly important in the manufacture of hats or other articles in light colours.

70 Moreover I prefer to so select the chlorine and the oxygen carrier that no solid precipitate is formed on the hair or wool in the course of the reaction, since such precipitates would greatly impair the lustre and the capacity of fulling or felting.

75 The same applies to the acidulating agent.

What I claim is:

80 1. A process for carroting animal hair and wool comprising the step of applying to the hair and wool aqueous solutions of hydrogen chloride and a chlorate and causing the two substances to react with each other in contact with the hair and wool.

85 2. A process of carroting animal hair and wool comprising the step of applying to the hair and wool an aqueous solution containing about three percent by weight of hydrogen chloride and about one percent by weight of a chlorate and causing the two substances to react with each other in contact with the hair and wool.

90 3. A process of carroting animal hair and wool comprising the step of applying to the hair and wool an aqueous solution of hydrogen chloride, a chlorate and oxalic acid and causing the hydrogen chloride and the chlorate to react with each other in contact with the hair and wool.

95 4. A process of carroting animal hair and wool comprising the step of applying to the hair and wool an aqueous solution containing about three percent by weight of hydrogen chloride and about one percent by weight of a chlorate and about one-half to six percent by weight of oxalic acid and causing the hydrogen chloride and the chlorate to react with each other in contact with the hair and wool.

100 5. A process for carroting animal hair and wool which consists in applying to the hair and wool an aqueous solution of hydrogen chloride and a solution of a substance selected from the group consisting of peroxide of hydrogen, persulphuric acid, persulphates, chloric acid, and chlorates.

105 In testimony whereof I have affixed my signature.

110 ERICH BÖHM.

115

120

125

130